

1

3,679,354

**PROCESS FOR THE MANUFACTURE OF HIGH BULK TEXTILE MATERIALS FROM POLY-ACRYLONITRILE**

Dietrich Hildebrand, Odenthal, and Karl Neufang, Cologne, Germany, assignors to Farbenfabriken Bayer Aktiengesellschaft, Leverkusen, Germany  
No Drawing. Filed Aug. 10, 1970, Ser. No. 62,654  
Claims priority, application Germany, Aug. 16, 1969,

P 19 41 706.2

Int. Cl. D06m 3/16

U.S. CL. 8—130.1

5 Claims

**ABSTRACT OF THE DISCLOSURE**

Process for the manufacture of high bulk textile materials of polyacrylonitrile by heat treatment of textile materials consisting of polyacrylonitrile fibre materials of different thermal shrinkability, characterised in that the heat treatment is carried out in chlorinated hydrocarbons which optionally contain small amounts of water and small amounts of emulsifiers.

The invention relates to a process for the manufacture of high bulk textile materials of polyacrylonitrile by heat treatment of textile materials consisting of polyacrylonitrile by heat treatment of textile materials consisting of nitrile fibre materials of different thermal shrinkability; the process is characterised in that the heat treatment is carried out in chlorinated hydrocarbons which optionally contain small amounts of water and small amounts of emulsifiers.

Processes are already known for bulking textile materials consisting of polyacrylonitrile fibre materials of different thermal shrinkability by treatment with boiling water or steam. The process according to the invention is distinguished from these known processes in that it yields high bulk materials which in handle, appearance and degree of cleanliness are superior to the high bulk textile materials manufactured according to the known processes, and furthermore in that the action of any brighteners contained in the textile materials is not impaired by the heat treatment carried out according to the invention. The main advantage of the process according to the invention however resides in the fact that the textile materials can be dyed from the same treatment bath immediately after the bulking process. The process according to the invention therefore represents a single-bath process for the bulking and dyeing of polyacrylonitrile fibre materials of different thermal shrinkability.

Possible chlorinated hydrocarbons for the process according to the invention are especially the chlorinated hydrocarbons with boiling points lying between 85 and 150° C., for example especially aliphatic chlorinated hydrocarbons, such as 1,1,1,2-tetrachlorethane, 1,1,2,2-tetrachloroethane, 1,1-dichloropropane, 1,2-dichloropropane, 1,3-dichloropropane, 1,1,1-trichloropropane, 1-chlorobutane, 2-chlorobutane, 1-chloro-2-methylpropane or 2-chloro-2-methylpropane and 1,1,1-trifluoropentachloropropane, but also aromatic hydrocarbons, such as chlorobenzene. Tetrachlorethylene and trichlorethylene have proved particularly suitable.

In some cases it has proved advantageous for the chlorinated hydrocarbon treatment baths to contain small amounts of water, say 0.01–2 percent by weight relative to the weight of the chlorinated hydrocarbons.

In order to distribute the water in the chlorinated hydrocarbons, it is appropriate to add commercially available emulsifiers to these. Amongst these emulsifiers, the following have proved particularly suitable: amines, amides and amine-oxides possessing at least 12 carbon atoms; am-

2

monium compounds possessing two hydrocarbon radicals with a total of at least 32 carbon atoms, such as N,N-dihexadecyl - N,N - dimethylammonium chloride, N-hexadecyl - N - oleyl - N,N - dimethylammonium methylsulphate and N,N - dihexadecyl - N - benzyl - N - methylammonium chloride; also, fatty acid ethanolamides and ethoxylation and/or propoxylation products of fatty alcohols, fatty amines, fatty acids, fatty acid amides, alkylphenols, aralkylphenols and arylphenols as well as their mixtures with one another. The emulsifiers are advantageously employed in an amount of 0.01–0.5 percent by weight relative to the weight of the chlorinated hydrocarbons.

In some cases it has furthermore proved advisable to add to the chlorinated hydrocarbons, additionally to the small amounts of water and emulsifiers, also small amounts, say 0.005–1 percent by weight, relative to the weight of the chlorinated hydrocarbons, of lower aliphatic carboxylic acids such as formic acid or acetic acid.

The polyacrylonitrile fibre materials of different thermal shrinkability to be bulked according to the process of the invention can be mixtures of fibre materials of different thermal shrinkability or bi-component fibres or bi-component filaments. The different thermal shrinkability can be based on a different thermal or thermal-mechanical pretreatment of the fibre materials or on a different modification of the polyacrylonitrile by various comonomers.

The polyacrylonitrile fibre materials to be bulked according to the invention can have been dyed with optical brighteners.

For dyeing the polyacrylonitrile fibre materials bulked according to the invention from the chlorinated hydrocarbon treatment baths, cationic dyestuffs can be used. These can be used in the form of salts, which are soluble in the chlorinated hydrocarbon, of dyestuff cations and anions of aliphatic or aromatic carboxylic, sulphonic or phosphonic acids possessing 4–30 carbon atoms, or in the form of water-soluble salts of dyestuff cations and anions of inorganic acids. These water-soluble salts are emulsified in the chlorinated hydrocarbon baths in the form of aqueous solutions.

As cationic dyestuffs there may for example be mentioned: methine, azomethine, hydrazone or azacyanine dyestuffs, dyestuffs of the diarylmethane or triarylmethane series, xanthene, thioxanthene, acridine, oxazine, thiazine and phenazine dyestuffs as well as cationic dyestuffs of the azo, anthraquinone or phthalocyanine series; by dyestuffs, there are also understood optical brighteners, for example optical brighteners of the stilbene, coumarine, azole or naphthalimide series.

Possible anions for the water-soluble dyestuff salts are above all the anions of inorganic acids, for example halide ions, such as the chloride, bromide or iodide ion, also the nitrate, perchlorate and bisulphate ion, and the anions which are derived from the sulphuric acid esters and sulphonic acids, such as the methylsulphate, ethylsulphate and toluenesulphonate ion.

Possible anions for the salts which are soluble in the chlorinated hydrocarbons are for example: the 2-ethylcaproate, laurate, oleate, linoleate, nonylphenol-tetraethyleneglycol-ether-propionate, 3-(nonylphenoxy)-propionate, nonyl-phenoxyacetate, tert.-butylbenzoate, hexahydrobenzoate, abietate, dodecylbenzenesulphonate and tetrapropylenebenzenesulphonate ion.

The amounts in which the dyestuffs optionally to be used are present in the dyebath can vary within wide limits depending on the desired depth of colour: 0.1–5 percent by weight of dyestuff, relative to the weight of the fibre material, have proved successful.

The process according to the invention is for example carried out in such a way that the fibre material to be bulked, which can be in the form of yarn, woven fabric or

knitted fabric or a made-up article manufactured therefrom, is treated for 5-60 minutes at 90-125° C. in a closed apparatus, for example a paddle apparatus or a drum dyeing apparatus, using a liquor ratio of 1:10-1:50, in the chlorinated hydrocarbons which optionally further contain small amounts of water, emulsifier and lower aliphatic carboxylic acids, such as formic or acetic acid. Following the bulking, the material is optionally dyed in the same bath by cooling the treatment bath to 80° C. adding the dyestuff and optionally small amounts of water and emulsifiers and dyeing for 30-90 minutes after addition of the dyestuff at 95-106° C.

Using the process according to the invention it is possible to bulk the textile materials of polyacrylonitrile fibre materials of different thermal shrinkability in a reproducible manner, whilst maintaining the optimum mechanical fibre properties and without impairing a previously applied brightening effect.

The parts indicated in the examples which follow are parts by weight.

#### EXAMPLE 1

100 parts of yarn of polyacrylonitrile fibres of different thermal shrinkability (60% thermally shrunk+40% unshrunk polyacrylonitrile fibres) are heated for 1 hour to 95° C. in 2400 parts of perchlorethylene in a closed apparatus. Thereafter the solvent is run out, adhering solvent is removed by centrifuging and the yarn is dried with warm air. A full, highly bulked yarn of very attractive handle is obtained, which shows a higher bulking effect and better handle properties than a corresponding yarn treated in an aqueous bath.

An equivalent bulking effect was also achieved by treating the yarn at 120° C. for 15 minutes.

#### EXAMPLE 2

100 parts of yarn of polyacrylonitrile fibres of different thermal shrinkability (60% thermally shrunk+40% unshrunk polyacrylonitrile fibres) in hank form are treated for 45 minutes at 95° C. in 1989 parts of perchlorethylene in a closed apparatus. Thereafter the bath is cooled to 80° C. and after addition of 11 parts of a dyestuff preparation consisting of:

6.6 parts of water,  
1.6 parts of oleyl alcohol eicosaglycol ether,  
0.8 part of oleic acid ethanolamide,  
1.0 part of di-octadecyl-dimethylammonium chloride,  
0.5 part of 60% strength acetic acid, and  
0.5 part of the dyestuff of formula



the whole is warmed to 98° C. and kept at this temperature for 1 hour with vigorous circulation of the liquor. The liquor is then run out, and the yarn is freed of the adhering solvent by centrifuging and is dried by blowing warm air over it; a highly bulked, greenish-tinged yellow, yarn is obtained which has a higher bulked volume than a yarn obtained from an aqueous treatment liquor.

#### EXAMPLE 3

5 100 parts of yarn of polyacrylonitrile fibres of different thermal shrinkability (70% thermally shrunk+30% thermally unshrunk polyacrylonitrile fibres) are heated for 30 minutes to 98° C. in a close apparatus in a bath consisting of:

1,980 parts of 1,1,1,2-tetrachlorethane,  
1.6 parts of oleyl alcohol eicosaglycol ether,  
0.8 part of oleic acid ethanolamide,  
0.4 part of 100% strength formic acid, and  
6.2 parts of water.

15 Thereafter the bath is cooled to 80° C. mixed with 11 parts of a dyestuff solution consisting of:

15.6 parts of the dyestuff of formula



20 25 30 35 58.8 parts of 1,1,1,2-tetrachlorethane and  
25.6 parts of butyrolactone,

and the whole heated to 98° C. over the course of 15 minutes.

After 1 hour's dyeing at this temperature the dyebath is run out. The yarn is rinsed with fresh 1,1,1,2-tetrachloroethane for 10 minutes at 45° C., subsequently centrifuged and dried by means of warm air. A bulked yarn dyed blue is obtained, having a greater bulked volume than a yarn obtained from an aqueous treatment liquor.

#### EXAMPLE 4

40 45 50 55 60 65 70 75 100 parts of yarn of polyacrylonitrile fibres of different thermal shrinkability (60% thermally shrunk+40% unshrunk polyacrylonitrile fibres) are heated for 5 minutes to 120° C. in a bath consisting of:

2,000 parts of perchlorethylene and

10 parts of mixture of

0.5 part of oleic acid ethanolamide,  
1 part of oleyl alcohol eicosaglycol ether,  
1 part of a compound of formula



0.5 part of glacial acetic acid and  
4 parts of water.

Thereafter the bath is cooled to 80° C. mixed with 4 parts of a mixture consisting of:

17.3 parts of the dyestuff salt of formula



57.7 parts of perchlorethylene and  
25.0 parts of butyrolactone,

70 75 warmed to 98° C. over the course of 15 minutes and kept at this temperature for 1 hour with vigorous agitation of the liquor. The liquor is then run out. The yarn is rinsed with fresh perchlorethylene for 5 minutes at room temperature and is subsequently centrifuged and freed of

the adhering solvent by blowing hot air over it. A highly bulked yarn, dyed golden yellow of soft handle is obtained, the manufacture of which requires less time than when using aqueous liquors.

We claim:

1. In the process of producing high bulk polyacrylonitrile textile materials by heat-treating textile materials consisting of polyacrylonitrile fiber materials of different thermal shrinkability, the improvement comprising conducting said heat-treatment in treating medium comprising chlorinated hydrocarbon, 0.01-2 percent by weight of water and 0.01-0.05 percent by weight of emulsifiers, relative to the weight of the chlorinated hydrocarbons.

2. The process of claim 1 in which the treating medium additionally contains 0.005-1 percent by weight of lower carboxylic acid, relative to the weight of said chlorinated hydrocarbon.

3. The process of claim 1 in which said heat-treatment is conducted for 5-60 minutes at 90-125° C.

4. The process of claim 1 in which said chlorinated hydrocarbon has a boiling point of 85 to 150° C.

5. The process of claim 1 in which said polyacrylonitrile textile materials are dyed in said treating medium immediately following heat-treatment.

#### References Cited

#### UNITED STATES PATENTS

|    |           |         |            |       |         |
|----|-----------|---------|------------|-------|---------|
| 10 | 3,481,685 | 12/1969 | White      | ----- | 8—130.1 |
|    | 3,514,249 | 5/1970  | Bullington | ----- | 8—130.1 |
|    | 2,789,340 | 4/1957  | Cresswell  | ----- | 28—76   |

GEORGE F. LESMES, Primary Examiner

J. CANNON, Assistant Examiner

U.S. CL. X.R.

8—1 W, 17, 114.6, 177 AB, 177 R

UNITED STATES PATENT OFFICE  
CERTIFICATE OF CORRECTION

Patent No. 3,679,354

Dated July 25, 1972

Serial No. 62,654

Inventor(s) Dietrich Hildebrand, et al.

It is certified that error appears in the above-identified patent and that said Letters Patent are hereby corrected as shown below:

| <u>Column</u>         | <u>Line</u>             | <u>Error</u>                                                                                                                                                                      |
|-----------------------|-------------------------|-----------------------------------------------------------------------------------------------------------------------------------------------------------------------------------|
| 1                     | 28                      | "nitrile by heat treatment of textile materials consisting of" should be deleted                                                                                                  |
| 2                     | 61                      | "3-" should be<br>---3- (---                                                                                                                                                      |
| 4                     | 6                       | "close" should be<br>---closed---                                                                                                                                                 |
| 5                     | 12<br>(Claim 1, line 7) | "0.05" should be<br>---0.5---                                                                                                                                                     |
| 3/4<br>(last formula) |                         | <p>CH<sub>3</sub><br/> <br/>CH<sub>2</sub>=<br/> <br/>CH<sub>3</sub></p> <p>CH<sub>3</sub> should be</p> <p>CH<sub>3</sub><br/> <br/>CH<sub>2</sub>=<br/> <br/>CH<sub>3</sub></p> |

UNITED STATES PATENT OFFICE  
CERTIFICATE OF CORRECTION

Patent No. 3,679,354 Dated July 25, 1972  
Serial No. 62,654  
Inventor(s) Dietrich Hildebrand, et al.

It is certified that error appears in the above-identified patent and that said Letters Patent are hereby corrected as shown below:

| <u>Column</u> | <u>Line</u> | <u>Error</u>                                     |
|---------------|-------------|--------------------------------------------------|
| 1             | 64          | "advantagesous" should read<br>--advantageous--. |

Signed and sealed this 6th day of March 1973.

(SEAL)  
Attest:

EDWARD M. FLETCHER, JR.  
Attesting Officer

ROBERT GOTTSCHALK  
Commissioner of Patents